

# United States Patent Office

2,739,060

Patented Mar. 20, 1956

1

2,739,060

## CHEMICAL SENSITIZATION OF PHOTOGRAPHIC EMULSIONS

Wesley G. Lowe, Jean E. Jones, and Harry E. Roberts, Rochester, N. Y., assignors to Eastman Kodak Company, Rochester, N. Y., a corporation of New Jersey

No Drawing. Application November 8, 1952,  
Serial No. 319,618

1 Claim. (Cl. 95—7)

This invention relates to photographic emulsions and more particularly to chemical sensitizers therefor.

It is well known that silver halide emulsions may be chemically sensitized with a variety of materials so as to increase the speed and generally the gamma of the emulsions as opposed to optical sensitizing in which the optical range of sensitivity is increased. Depending upon the materials and methods employed, it is generally regarded that chemical sensitization results in either the formation of silver sulfide on the surface of the silver halide crystal or results in the formation of small amounts of silver from the reduction of silver halide, which effect may be in addition to the former effect usually known as sulfur sensitizing. The present invention is concerned primarily with chemical sensitization apparently of the latter type.

It has been proposed to use organic and inorganic sulfides in photographic emulsions to increase the sensitivity thereof. The compounds are generally regarded as imparting the above-mentioned type of sulfur sensitizing resulting from the formation of silver sulfide nuclei on the silver halide grains. In the Lowe et al. U. S. Patent 2,521,926 granted September 12, 1950, have been proposed a group of organic sulfur-containing compounds which have little or no activity as sulfur sensitizing agents but which appear to depend for their sensitizing effect upon enlargement of the silver sulfide nuclei by deposition of silver thereon through reduction of silver halide. Whatever the mechanism involved, the sensitizing effect is readily distinguishable from ordinary sulfur sensitizing and when employed in conjunction with sulfur sensitizing can be separately evaluated.

We have now found that when silver halide emulsions are sensitized with a mixture of a sulfur sensitizing agent, a gold salt sensitizing agent and the organic sulfide sensitizing agents of the Lowe et al. invention, a speed increase is obtained greater than that expected from the individual effects of the sensitizing agents and greater than that expected from the combined effect of any two of the three types of sensitizing agents.

Therefore, one object of our invention is to provide chemically sensitized emulsions of enhanced light sensitivity. Another object is to provide emulsions having sensitivity enhanced by the combined effect of sulfur, gold and certain organic sulfide compounds. A further object is to provide the methods of augmenting emulsion sensitivity utilizing the novel combination of sensitizing agents. Another object is to provide photographic elements in which the novel emulsions are useful. Further objects of our invention will become apparent from consideration of the following description.

The objects of our invention are accomplished by the incorporation into silver halide emulsions of a mixture of (A) a sulfur-sensitizing agent such as disclosed in Sheppard U. S. Patents 1,574,944 granted March 2, 1926, and 1,623,499 granted April 5, 1927, e. g. thiourea, di-o-tolyl thiourea, allyl isothiocyanate, thiocarbanilide, sodium thiosulfate, thioacetamide and allyl thiourea, (B) a gold salt sensitizing agent such as disclosed in Waller

2

and Dodd U. S. Patent 2,399,083 e. g. gold chloride, potassium chloroaurate or an alkali metal aurothiocyanate such as potassium aurothiocyanate, and (C) either bis-( $\beta$ -aminoethyl) sulfide ( $\text{NH}_2\text{CH}_2\text{CH}_2\text{S}$ )<sub>2</sub>S and its water-soluble salts obtained from non-desensitizing acids such as the acetates, carbonates, sulfates and hydrochloride salts, or bis-( $\gamma$ -diethyl aminopropyl) disulfide



10 at any stage in their preparation but preferably before digestion is complete.

The quantity of sulfur, gold and organic sulfide sensitizing agents used in the emulsions is not especially critical and can be varied from the optimum amounts indicated in the following examples.

The sensitizing agents are incorporated into the emulsions at any stage in their preparation but preferably before digestion is complete. That is, the emulsion can first be sensitized with a sulfur sensitizing agent and a gold salt sensitizing agent and then one of the organic sulfide sensitizing agents indicated, or the addition of the organic sulfide compound can be made prior to the addition of the gold salt sensitizing compound. However, it is preferred to partially digest the emulsion in the presence of the selected sulfur and gold sensitizing agents and to finish the emulsion by digesting it further after addition of the organic sulfide compound since the greatest speed increases are obtained in this manner. One rather unexpected feature of our invention resides in the fact that while the emulsions can be digested to optimum sensitivity in the presence of the sulfur and gold sensitizing agents, further digestion after addition of the organic sulfide compound does not cause any appreciable increase in fog.

35 The following examples illustrate means for carrying out our invention:

### Example 1

A. In a positive type of silver bromoiodide emulsion were incorporated 20 milligrams of allyl thiourea per mol 40 of silver halide and 2 milligrams of potassium chloroaurate per mol of silver halide and the emulsion was digested for 61 minutes at 62° C. A sample of the emulsion was coated onto film base.

B. To a sample of emulsion A above were added 400 milligrams of bis-( $\beta$ -aminoethyl) sulfide dihydrochloride per mol of silver halide and the emulsion was digested for 20 minutes at 40° C. before coating on film base.

C. An emulsion was prepared as in B except using 600 milligrams of the sulfide per mol of silver halide.

50 The coatings of emulsions A, B and C were exposed in the sensitometer and developed for 3 minutes in the following developer:

|                                  |       |      |
|----------------------------------|-------|------|
| Water, about 125° F. (50° C.)    | cc    | 500  |
| p-Methylamino-phenol sulfate     | grams | 2.2  |
| Sodium sulfite, desiccated       | do    | 96.0 |
| Hydroquinone                     | do    | 8.8  |
| Sodium carbonate, desiccated     | do    | 48.0 |
| Potassium bromide                | do    | 5.0  |
| 60 Cold water to make 1.0 liter. |       |      |

### Example 2

D. To a fine-grained gelatino silver bromoiodide emulsion were added a sulfur sensitizing agent such as described above and a gold salt sensitizing agent such as described above. The emulsion was then digested to optimum sensitivity and a sample coated on film.

E. A portion of the digested emulsion of D was treated with 0.400 gram of bis-( $\beta$ -aminoethyl) sulfide per mol of silver halide and the emulsion was held at 40° C. for 30 minutes, then coated on to film.

F. A portion of the digested emulsion of D was treated with 0.800 gram of bis-( $\beta$ -aminoethyl) sulfide per mol

of silver halide and the emulsion was held at 40° C. for 30 minutes, then coated on to film.

The coated films of emulsions D, E and F were then exposed in an Eastman type Ib sensitometer and processed for 5 minutes in a developer of the following composition:

|                             |        |      |
|-----------------------------|--------|------|
| Water                       | liters | 1    |
| p-Methylaminophenol sulfate | grams  | 0.3  |
| Hydroquinone                | do     | 6.0  |
| Sodium sulfite (dry)        | do     | 38.0 |
| Sodium bisulfite            | do     | 1.2  |
| Sodium carbonate (dry)      | do     | 19.0 |
| Potassium bromide           | do     | 0.9  |
| Citric acid                 | do     | 0.7  |

The sensitometric characteristics of the coatings of Examples 1 and 2 are tabulated in the following table:

| Sample | Sensitizer          | 10/i Speed | Gamma | Fog  |
|--------|---------------------|------------|-------|------|
| A      | Sulfur+gold         | 5.4        | 3.28  | 0.04 |
| B      | Sulfur+gold+sulfide | 8.6        | 3.48  | 0.04 |
| C      | do                  | 9.4        | 3.50  | 0.04 |
| D      | Sulfur+gold         | 37         | 2.27  | 0.02 |
| E      | Sulfur+gold+sulfide | 43         | 2.51  | 0.03 |
| F      | do                  | 46         | 2.47  | 0.03 |

The substantial speed increase imparted to the sulfur and gold sensitized emulsions by addition of the organic sulfide sensitizing agent is apparent from the date.

In the manner of the above example, other sulfur sensitizing agents, gold salt sensitizing agents and bis-( $\beta$ -aminoethyl) sulfide or bis-( $\gamma$ -diethyl aminopropyl) disulfide can be used in combination for sensitizing silver halide emulsions and results comparable to those indicated above can be expected.

In the manner of the above examples, many types of

silver halide emulsions can be treated with the novel combination of sulfur, gold and organic sulfide sensitizing agents. The novel sensitizers may, in general, be employed in hydrophilic colloid emulsion vehicles; for example, gelatin, polyvinyl alcohol, partially hydrolyzed cellulose ester, such as cellulose acetate and copolymers of polyvinyl alcohol. The sensitizers are suitable for the well known types of silver chloride, silver bromide and silver iodide emulsions and emulsions containing mixtures of these halides, containing the usual emulsion addenda such as antifoggants, spreading agents, coupler compounds, etc. Such emulsions are suitable to use in forming single as well as multilayer film useful in color photography which customarily include on a support two or more emulsion layers sensitized to different regions of the visible spectrum and may or may not contain coupler compounds. According to our invention such color films carry at least one emulsion layer containing the mentioned combination of sensitizing agents.

Our invention having been described, we would have it understood that the preceding description is by way of example only and that our invention is to be taken as limited only by the scope of the appended claim.

#### What we claim is:

A light-sensitive photographic emulsion comprising silver halide sensitized with a sulfur sensitizing agent, a gold salt sensitizing agent and bis-( $\gamma$ -diethylaminopropyl) disulfide.

#### References Cited in the file of this patent

#### UNITED STATES PATENTS

- |           |                   |                |
|-----------|-------------------|----------------|
| 2,399,083 | Waller et al.     | Apr. 23, 1946  |
| 2,521,926 | Lowe et al.       | Sept. 12, 1950 |
| 2,540,086 | Baldsieben et al. | Feb. 6, 1951   |
| 2,597,856 | Damschroder       | May 27, 1952   |